

March 11, 1969

H. L. WHEATON

**3,432,294**

COBALT-BASE ALLOY

Filed April 21, 1965

Sheet 1 of 4

**FIG. 1**



**FIG. 2**



INVENTOR

HAROLD L. WHEATON  
BY *Francis J. Mulligan Jr.*  
ATTORNEY

March 11, 1969

H. L. WHEATON

3,432,294

COBALT-BASE ALLOY

Filed April 21, 1965

Sheet 2 of 4



FIG. 3

STRESS - PSI

INVENTOR.  
HAROLD L. WHEATON

BY

*Harold L. Wheaton*

ATTORNEY

March 11, 1969

H. L. WHEATON

3,432,294

COBALT-BASE ALLOY

Filed April 21, 1965

Sheet 3 of 4

FIG. 4



STRESS FOR 1000 HOUR LIFE - PSI

INVENTOR  
HAROLD L. WHEATON  
BY *Harold L. Wheaton Jr.*

ATTORNEY

March 11, 1969

H. L. WHEATON

3,432,294

COBALT-BASE ALLOY

Filed April 21, 1965

Sheet 4 of 4

FIG. 5



INVENTOR.  
HAROLD L. WHEATON

BY *Harold L. Wheaton*

ATTORNEY

3,432,294

## COBALT-BASE ALLOY

Harold L. Wheaton, Rolling Meadows, Ill., assignor to  
Martin-Marietta Corporation, New York, N.Y., a corpora-  
tion of Maryland

Filed Apr. 21, 1965, Ser. No. 449,825

U.S. Cl. 75—171  
Int. Cl. C22c 19/02

8 Claims

## ABSTRACT OF THE DISCLOSURE

An alloy suitable for use under load at high temperatures and having an excellent combination of engineering characteristics. The alloy is a carbide-hardened cobalt-base material containing critical, related amounts of carbon, chromium, nickel, tungsten, tantalum, titanium and zirconium.

The present invention relates to alloys and, more particularly, to cobalt-base, carbide-hardened alloys especially adapted for use at elevated temperatures at high stress.

For a number of years during the development of the gas turbine engine for aircraft and stationary usage, it has been the goal to produce stronger and stronger cobalt-base alloys. Now that the race for brute strength of cobalt-base alloys is being won by achievement of useful strengths at temperatures of the order of 80% of the absolute melting temperature of the alloys in question, more and more attention is being directed to the need for the development of other highly useful and necessary characteristics in useful high-strength alloys.

One of the problems which has plagued developers of cobalt-base, carbide-hardened alloys is the problem of producing a strong alloy which not only is relatively metallurgically stable at temperatures at the extremely high ranges of 1800° F. and higher, but also is resistant to drastic embrittlement resulting from exposure to lower temperatures, e.g. temperatures about 1000° F. to about 1600° F. It is well recognized in general that exposure to temperatures above the recrystallization range will alter the metallurgical characteristics of an alloy, such alteration being due, at least in part, to grain growth. At lower temperatures other changes can occur. In cobalt-base, carbide-hardened alloys of the kind in question, hardness increases are experienced when the alloys are subjected for prolonged periods of time at temperatures of the order of 1300° F. to 1600° F. For example, a prior art, precision-cast, carbide-hardened cobalt-base alloy might exhibit an as-cast hardness of 40 R<sub>c</sub> (Rockwell C units) which hardness could increase to 50 R<sub>c</sub> upon exposure for about 48 hours at 1500° F. Should such an increase in hardness accrue during engine operation, for example during operation of a gas turbine engine incorporating water injection, an increase in hardness along with an inherent decrease in ductility and increase in brittleness could prove to be a fatal deficiency for the engine part in question. It is, therefore, very important that a cobalt-base carbide-hardened alloy should exhibit as low an as-cast hardness as is compatible with achieving useful levels of strength at elevated temperatures.

Mechanical characteristics, other than brute strength at extremely high temperatures, which are necessary for a successful gas turbine alloy include good high temperature creep strength and rupture ductility, good high temperature oxidation resistance, good thermal conductivity and acceptable room-temperature strength and ductility. All in all, a successful gas-turbine alloy of the kind in question must meet and pass many tests in order to be practically and commercially useful. As far as I am aware,

no one has heretofore provided the art with an alloy having such an advantageously high combination of engineering characteristics, as is exhibited by the alloy of the present invention, wherein a substantial balance of characteristics is attained without substantial sacrifice of any particular feature.

It has now been discovered that by means of a special control of alloying elements within specially controlled and, advantageously, interrelated ranges a novel carbide-hardened, cobalt-base casting alloy can be produced having an advantageous balance of engineering characteristics and possessing highly enhanced practical utility.

It is an object of the present invention to provide a novel cobalt-base alloy.

It is another object of the present invention to provide a novel cobalt-base, carbide-hardened alloy.

A still further object of the present invention is to provide precision-cast engineering structures made of a novel cobalt-base, carbide-hardened alloy.

Another object of the present invention is to provide novel, precision-cast gas-turbine structures made of a novel cobalt-base, carbide-hardened alloy.

An additional object of the present invention is to provide a process for the production of a novel alloy and for the production of engineering structures, e.g. gas-turbine structures comprised thereof.

Other objects and advantages will become apparent from the following description taken in conjunction with the drawing in which:

FIGURE 1 is a sketch depicting the as-cast microstructure of an alloy in accordance with the present invention, as viewed at about 250 power magnification;

FIGURE 2 is a sketch depicting the as-cast microstructure of a useful prior art alloy, as viewed at about 250 power magnification;

FIGURE 3 is a graph showing life-to-rupture in hours for an alloy of the present invention under various loads in pounds per square inch (p.s.i.) at various temperatures between and including 1400° F. and 2000° F.;

FIGURE 4 is a graph showing the interrelation between stress for 100 hour life (in p.s.i.) and temperature (in degrees Fahrenheit) for an alloy of the present invention and some prior art alloys; and

FIGURE 5 is a graph illustrating the creep behavior of any alloy in accordance with the present invention, as compared to the creep behavior of some prior art alloys.

Generally speaking, the present invention is directed to a cobalt-base, carbide-hardened alloy containing in weight percent about 0.6% carbon, about 18% to about 24% chromium, about 7% to about 15% nickel, about 6% to about 9% tungsten, about 2% to about 5% tantalum, about 0.1% to about 0.5% titanium, about 0.1% to about 1% zirconium with the balance being essentially cobalt together with impurities and incidental elements normally associated with cobalt-base alloys. The alloy of the present invention is particularly adapted to be formed by precision casting into engineering structures useful at elevated temperatures such as encountered in gas turbines.

Among the incidental elements which may be present in the alloy of the present invention are up to about 3% iron, up to about 0.5% each of manganese and silicon, up to about 0.1% boron, up to about 0.2% mischmetal (a mixture of rare earth metals), up to about 2% of columbium and up to about 2% of molybdenum. It is advantageous to maintain the impurity elements sulfur, hydrogen, lead, tin and others of like activity at as low levels as possible in order to avoid the deleterious effects caused by interstitial infiltration of the crystal lattice by hydrogen and the like and the formation of low melting phases by lead, tin, sulfur, and the like.

When producing the alloy of the present invention, it is

highly advantageous to employ vacuum melting wherein the alloying elements cobalt, chromium, nickel, tungsten and carbon are melted together under a high vacuum and held in the molten condition thereunder until deoxidation has been completed. Subsequent to completion of said deoxidation tantalum is added to the molten metal followed by titanium and zirconium. When alloying is completed, the melt is cast either into bars suitable for remelting or directly into finished shapes by means of suitably shaped molds, e.g. molds produced by investing a fugitive model in a ceramic matrix. Advantageously casting as well as melting is carried out under a high vacuum. Alternatively, one can melt and cast under an inert atmosphere such as argon. However, when such is done, it is necessary to employ deoxidizing agents, such as silicon, aluminum and rare earth elements in order to kill the melt prior to the addition of tantalum, titanium and zirconium.

When melting under vacuum conditions, carbon acts not only as an alloying ingredient but also as a deoxidizer. Thus when melting in the usual manner as employed under vacuum, i.e. in a high frequency induction furnace, it is necessary to carefully adjust the carbon content of the original charge to produce a final carbon content within the range of about 0.4%, to about 0.7%, advantageously about 0.5% to about 0.7%. In order to avoid loss of strength and oxidation resistance, one should avoid chromium contents below about 19%. On the other hand, use of chromium contents above about 23% can in certain instances lead to brittleness in the alloy. It is advantageous for all round good characteristics (especially low as-cast hardness and enhanced resistance to oxidation) to employ about 10% nickel in the alloy. However, one can use plus or minus 2% as a practical, efficacious and advantageous range for this element. Nickel contents in excess of 15% drastically lower rupture strength.

The carbide formers, tungsten, tantalum, titanium and zirconium, are advantageously employed in amounts of about 7% tungsten, about 3.5% tantalum, about 0.2% titanium and about 0.5% zirconium in conjunction with about 0.6% carbon. When used in these amounts, the carbide-forming elements, in conjunction with the carbon tend to produce a stable, dispersed carbide phase in the cobalt-chromium-nickel matrix which stable, dispersed phase does not form a continuous network throughout the matrix. The importance of this type of stable structure, which is depicted in FIGURE 1 of the drawing, is the fact that a high basic thermal conductivity of the alloy due to a continuous metal matrix is achieved upon casting and remains substantially unimpaired even after prolonged exposure to temperatures of about 1400° F. to about 1900° F. Thus the alloy of the present invention, when cast into objects such as guide vanes for gas turbine engines, permits the efficient transfer of heat from locally superheated portions to cooler portions thus prolonging the useful life of the object. In prior art alloys having somewhat higher carbon contents in superficially similar compositions, massive, semi-continuous, carbide phases, as depicted in FIGURE 2, are formed. Because the thermal conductivity of massive, semi-continuous carbide phases is relatively low compared to the thermal conductivity of a cobalt alloy matrix and because heat transfer is slowed at phase boundaries, objects made of prior art alloys having a microstructure such as depicted in FIGURE 2 are likely to fail at hot spots especially when

stress is concentrated in areas where hot spots can develop. Further, massive carbide structures, especially in semi-continuous or continuous form, provide brittle areas through which stress-induced cracks can propagate rapidly.

It is to be noted that among themselves, the carbide-forming elements are advantageously interrelated such that the amount of tungsten in weight percent is about twice the amount of tantalum in weight percent, the weight percent of zirconium is about 2.5 times the weight percent of titanium and the sum of the weight percent zirconium plus twice the weight percent titanium is less than about 1.5%. While these interrelations are somewhat empirical in nature and can, in practice, be varied somewhat within the alloy or range limits set forth hereinbefore, experimental experience has shown that one cannot ignore these interrelations and still achieve a commercially advantageous alloy. Generally, as indicated by the mean of the alloy ranges set forth hereinbefore, it is advantageous that ratio of the atom percent of carbon to the total atom percent of carbide-forming elements, to wit, tungsten, tantalum, zirconium and titanium be maintained at about 0.72 in order to attain high creep rupture characteristics. The aforementioned advantageous ratios of tungsten to tantalum and zirconium to titanium serve the same purpose. On the other hand, the aforementioned maximum summation of percentages of zirconium plus titanium is maintained for the purpose of assuring good oxidation resistance at elevated temperatures.

For purposes of the present invention it is to be noted that molybdenum is not the equivalent of tungsten and columbium as a substitute for a part of the required tantalum. While the alloys of the present invention can contain up to about 2% by weight of molybdenum as an impurity or incidental element, this element is not a substitute for the required amount of tungsten. Where oxidation resistance is not a prime factor, one can employ columbium as a substrate for a part of the required tantalum on a 1/2 to 1 by weight basis. However, in the usual case this is not recommended. Usually, columbium in amounts up to 0.5% by weight can be present in the alloy as an impurity or incidental element associated with tantalum. In like manner small amounts of hafnium can be present in the alloy of the present invention as an element introduced in association with zirconium.

For the purpose of giving those skilled in the art a better understanding of the invention and/or a better appreciation of the advantages of the invention, the following illustrative examples are given:

50

#### Example

Alloys (hereinafter referred to as alloy No. 1) containing 0.0% carbon, 21.5% chromium, 10% nickel, 7% tungsten, 3.5% tantalum, 0.20% titanium, 0.5% zirconium with the balance essentially cobalt is melted under vacuum in a high-frequency induction furnace and poured at 2800° F. under vacuum into molds to produce tensile test bars, stress-rupture test bars, oxidation test specimens and airfoil-section test specimens for thermal shock tests.

Additional alloy compositions comprising alloys 2 and 3 (within the invention) and alloys A to H (outside the invention) and having compositions in weight percent, as set forth in Table I, were made in the same manner as the alloy of the example.

TABLE I

| Alloy No. | Percent C | Percent Cr | Percent Ni | Percent Co | Percent W | Percent Ta | Percent Ti | Percent Zr | Other, Cb |
|-----------|-----------|------------|------------|------------|-----------|------------|------------|------------|-----------|
| 2-----    | 0.52      | 20.8       | 11.9       | Bal.       | 7.8       | 4.3        | 0.16       | 0.41       | -----     |
| 3-----    | 0.51      | 21.7       | 8.1        | Bal.       | 5.1       | 2.6        | 0.22       | 0.59       | -----     |
| A-----    | 0.53      | 21.4       | -----      | Bal.       | 7.1       | 3.6        | 0.16       | 0.56       | -----     |
| B-----    | 0.51      | 21.7       | -----      | Bal.       | 6.2       | 3.1        | 0.37       | 1.3        | -----     |
| C-----    | 0.55      | 21.3       | -----      | Bal.       | 8.4       | 4.2        | -----      | 0.10       | -----     |
| D-----    | 0.30      | 20.9       | 8.2        | Bal.       | 5.6       | 2.8        | 0.22       | 0.49       | -----     |
| E-----    | 0.60      | 25         | 10         | Bal.       | 7.2       | -----      | 0.18       | 0.52       | -----     |
| F-----    | 0.85      | 21.5       | -----      | Bal.       | 10        | 9          | -----      | 0.15       | -----     |
| G-----    | 0.45      | 21         | -----      | Bal.       | 11        | -----      | -----      | -----      | 1.75      |
| H-----    | 0.50      | 25         | 10         | Bal.       | 7.5       | -----      | -----      | -----      | -----     |

The data set forth in Table II which pertains to the alloys of the example and Table I shows that the lives to rupture at 2000° F. and 8000 pounds per square inch (p.s.i.) of alloys of the present invention are at least substantially equivalent to the lives to rupture of alloys outside the present invention. Further, the stress (in p.s.i.) for 100 hour life versus temperature curves for the alloy of the example and alloys Nos. F, G, and H are depicted in FIGURE 4 of the drawing. These curves show that the alloy of the present invention exhibits unexpectedly superior strength at temperatures in excess of about 1550° F. when compared to alloys (i.e. alloys F, G, and H) previously suggested for use in gas turbines and other structures subjected in use to high temperatures.

TABLE II

| Alloy No. | Temperature<br>(° F.) | Stress<br>(p.s.i.) | Life<br>(Hours) | Elongation,<br>percent<br>(1/2" gauge<br>length) |
|-----------|-----------------------|--------------------|-----------------|--------------------------------------------------|
| 1-----    | 2,000                 | 8,000              | 11.1            | 7                                                |
| 2-----    | 2,000                 | 8,000              | 79.0            | 11                                               |
| 3-----    | 2,000                 | 8,000              | 77              | 11                                               |
| A-----    | 2,000                 | 8,000              | 109.1           | 10                                               |
| B-----    | 2,000                 | 8,000              | 135.4           | 18                                               |
| C-----    | 2,000                 | 8,000              | 51.5            | 7                                                |
| D-----    | 2,000                 | 8,000              | 20.2            | 28                                               |
| E-----    | 2,000                 | 8,000              | 43.2            | 20                                               |
| F-----    | 2,000                 | 8,000              | 30.5            | 13                                               |
| G-----    | 2,000                 | 8,000              | 17.8            | 13                                               |
| H-----    | 2,000                 | 8,000              | 5.0             | (1)                                              |

<sup>1</sup> Not available.

Alloy C, which contains no titanium and only a trace of zirconium, and Alloy E, which contains 1.8% columbium substituted for 3.6% tantalum, are considerably weaker than the alloys of this invention (i.e., 1, 2, and 3) as are the prior art alloys, F, G, and H.

Alloys substantially of the composition of alloy No. 1 (that is, alloys made to conform to the chemistry of alloy No. 1 but exhibiting the normal variations in chemistry occurring in foundry practice) exhibit lives to rupture at various temperatures and under differing stresses as indicated by the linear plots on the graph depicted in FIGURE 3 of the drawing. A comparison of FIGURES 3 and 4 of the drawing shows, for example, that at 1800° F., the life-to-rupture of alloy No. 1 can be expected to be about 4 times as great as the life-to-rupture of alloy No. F when both are tested under a load of about 14,500 p.s.i. For the sake of completeness, it is to be noted that the test data set forth in Table II and in FIGURE 4 of the drawing was obtained by employing the standard test for life-to-rupture, as described in ASTM E8-61T and by using as-cast specimens 0.25 inch diameter and 1.4 inches in length exclusive of that length required for gripping. An additional pertinent point is, that at temperatures in excess of about 1600° F., the creep behavior of alloys of the present invention differs substantially from that of prior cobalt-base alloys suggested for use at 1800° F. and higher. FIGURE 5 of the drawing illustrates this point showing the creep behavior of an alloy in accordance with the invention when tested at 2000° F. under a load of 8000 p.s.i. as compared to the creep behavior of comparably tested Alloys Nos. F and G. FIGURE 5 shows that under the test conditions specified, the alloy of the present invention exhibits a well-defined, low second stage creep rate as compared to the ill-defined, high second stage creep rate of prior alloys suggested for use at temperatures in excess of about 1600° F.

In addition to rupture strength, a basic requirement for any high temperature structural material is oxidation resistance. Materials possessing inadequate oxidation resistance must be coated which adds to the cost and lowers reliability. The oxidation behavior of the alloys listed in Table I is shown in Table III. Alloys with weight gains under 5 mg./cm.<sup>2</sup> and having adherent scales can be considered oxidation resistant while those having weight gains over 5 mg./cm.<sup>2</sup> or scales that spall do not have sufficient oxidation resistance to be used in the uncoated condition at 2000° F.

TABLE III

| Alloy No. | Temperature<br>(° F.) | Time<br>(hours) | Specific<br>weight gain<br>(mg./cm. <sup>2</sup> ) | Scale appearance and<br>adherence |
|-----------|-----------------------|-----------------|----------------------------------------------------|-----------------------------------|
| 5 1-----  | 2,000                 | 100             | 1.4                                                | Thin and adherent.                |
| 2-----    | 2,000                 | 100             | 2.8                                                | Do.                               |
| 3-----    | 2,000                 | 100             | About 2.5                                          | Do.                               |
| A-----    | 2,000                 | 100             | 3.1                                                | Thin but some light<br>spalling.  |
| B-----    | 2,000                 | 100             | 14.0                                               | Thick, heavy scaling.             |
| C-----    | 2,000                 | 100             | 2.5                                                | Thin but some light<br>spalling.  |
| 10 E----- | 2,000                 | 100             | 10.0                                               | Thick, moderate spal-<br>ling.    |
| F-----    | 2,000                 | 100             | 2.5                                                | Thin and adherent.                |
| G-----    | 2,000                 | 100             | 34.0                                               | Very thick, heavy spal-<br>ling.  |
| H-----    | 2,000                 | 100             | (1)                                                |                                   |

15 <sup>1</sup> Not available.

A comparison of alloy A with alloy 1 indicates the beneficial effect of nickel on oxidation resistance while a comparison of alloy B and alloy 1 shows the deleterious effect of high zirconium plus titanium. Alloy C has fairly good oxidation resistance but relatively low creep rupture strength because of the absence of zirconium and titanium. Alloy E, which contains the atomic equivalent of columbium substituted for tantalum, has poor oxidation resistance even with a chromium content of 25% and the addition of 10% nickel. The oxidation data for prior art alloys F and G are included for comparative purposes although their rupture strengths are such that oxidation data are somewhat academic.

Another novel aspect of the alloys of the present invention, when compared with some other cobalt-base, carbide-hardened alloys, is shown by the as-cast and aged hardness data in Rockwell C units (R<sub>c</sub>) set forth in Table IV.

TABLE IV

| Alloy No. | As-cast<br>hardness (R <sub>c</sub> ) | Hardness after<br>48 hours at<br>1,500° F. (R <sub>c</sub> ) |
|-----------|---------------------------------------|--------------------------------------------------------------|
| 40 1----- | 32                                    | 42                                                           |
| 2-----    | 28                                    | 41                                                           |
| 3-----    | 31                                    | 41                                                           |
| A-----    | 36                                    | 46                                                           |
| B-----    | 36                                    | 42                                                           |
| C-----    | 36                                    | 46                                                           |
| D-----    | 26                                    | 35                                                           |
| E-----    | 31                                    | 43                                                           |
| F-----    | 40                                    | 50                                                           |
| G-----    | 37                                    | 44                                                           |
| H-----    | 34                                    | 42                                                           |

A comparison of alloy A and alloy 1 shows the necessity of using nickel to control the as-cast and aged hardnesses in order to avoid undesirable embrittlement. Alloy D, having a low carbon content, illustrates the fact that relatively low hardnesses can be attained by lowering the carbon content. However, as shown in Table II, the low carbon content results in a low life-to-rupture at 2000° F. Alloy F, on the other hand, illustrates the fact that high hardnesses in the as-cast and aged conditions do not necessarily result in a high life-to-rupture. Table II shows that alloy F exhibits a life-to-rupture which is not significantly different from the life-to-rupture of alloy D even though there is a marked difference in both the carbon contents and the hardnesses of these alloys. Since, as is shown, cobalt-base, carbide-hardened alloys increase in hardness by an increment of about 8 to 10 Rockwell C units by virtue of being subjected to temperatures of the order of 1500° F. for about 48 hours, the lower as-cast hardness of alloys in accordance with the invention indicates highly enhanced utility especially when viewed in light of the data set forth in Tables II and III. A composite view of the data of Tables II, III and IV shows that alloys of the present invention exhibit a unique combination of strength, oxidation resistance, and resistance to embrittlement not present in alloys outside the invention or alloys of the prior art.

A further measure of the unique utility of the alloys of the present invention as compared to other cobalt-

base, carbide-hardened alloys is demonstrated in the data set forth in Table V, which data relates to the results of a thermal fatigue-deflection test. The thermal fatigue-deflection test comprises subjecting an airfoil shaped sample 2 inches long and 1 inch wide with a maximum thickness of  $\frac{1}{8}$  inch to repeated cycles wherein the sample is heated to about 2000° F. for 1.5 minutes and then allowed to cool for 0.5 minute in an air blast containing water spray. This heating and cooling cycle is repeated until 500 cycles are complete.

Table V

| Alloy No.: | Mils deflection after 500 cycles |
|------------|----------------------------------|
| 1          | 31                               |
| F          | 96                               |
| G          | 26                               |

The data in Table V shows that alloys of the present invention exhibit unique utility when subjected to thermally induced stress. Thermally induced stress and fatigue resulting therefrom is a day-to-day hazard which must be faced by any alloy used for any part in the hot-zone of an aircraft gas turbine engine. Basically the data in Table V shows that the thermal conductivity as measured by resistance-to-deflection of the alloys of the present invention is significantly better than the thermal conductivity of the v. prior art, cobalt-base, carbide-hardened alloy F and essentially equivalent to prior art alloy G which, as mentioned previously, has poor oxidation resistance and low creep-rupture strength. This large difference is primarily due to the metallographic factors discussed hereinbefore which, in turn, result from the metallurgical and elemental makeup of the novel alloys.

The alloys of the present invention also exhibit excellent room temperature (77° F.) and high temperature tensile characteristics are demonstrated by the data set forth in Table VI relating to alloy No. 1.

TABLE VI

| Temperature       | Ultimate tensile strength (K s.i.) | Yield strength, percent offset (K s.i.) | Percent elongation | Percent reduction in area |
|-------------------|------------------------------------|-----------------------------------------|--------------------|---------------------------|
| R.T. <sup>1</sup> | 115                                | 93                                      | 3.5                | 5.0                       |
| R.T. <sup>1</sup> | 110                                | 84                                      | 3.0                | 3.2                       |
| 600° F.           | 85.9                               | 58.3                                    | 4.5                | 7.8                       |
| 1,200° F.         | 72.6                               | 52.4                                    | 5.0                | 10                        |
| 1,400° F.         | 71.5                               | 48.3                                    | 5.5                | 10                        |
| 1,600° F.         | 67.8                               | 45.7                                    | 7.0                | 13                        |
| 1,800° F.         | 44.7                               | 28.6                                    | 14                 | 25                        |
| 1,960° F.         | 28.0                               | 14.7                                    | 29                 | 42                        |

<sup>1</sup> R.T. = Room temperature.

Alloys of the present invention (the compositions of which are expressed herein in terms of percent by weight) are highly useful for the manufacture of precision cast objects including nozzle guide vanes, turbine blades, and after burner components. Where necessary, the alloys of the present invention can be machined in the manner common to all carbide-hardened, cobalt-base alloys, i.e. by grinding.

Although the present invention has been described in conjunction with advantageous embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. A carbide-hardened alloy consisting essentially of, in weight percent, about 0.4% to about 0.7% carbon, about 18% to about 24% chromium, about 7% to about 15% nickel, about 6% to about 9% tungsten, about 2% to about 5% tantalum, about 0.1% to about 0.5% titanium, about 0.1% to about 1% zirconium with the balance being essentially cobalt together with impurities and incidental elements normally associated with cobalt-base alloys, said alloy being characterized by a high combination of engineering characteristics necessary for structures used under stress at elevated temperatures in oxidizing atmospheres.

2. A precision cast alloy object made of the alloy of claim 1.

3. A precision cast, gas turbine structure made of the alloy of claim 1.

4. An alloy as in claim 1, wherein the carbon content is at least about 0.5%, the chromium content is at about 19% and the nickel content is about 10%.

5. An alloy as in claim 1 wherein the amounts of the elements: carbon, tungsten, tantalum, titanium and zirconium are related such that the weight percent of tungsten is about twice the weight percent of tantalum, the weight percent of zirconium is about 2.5 times the weight percent of titanium, and the ratio of the atomic percent of carbon to the total of the atomic percents of tungsten, tantalum, zirconium and titanium is about 0.72.

6. A cobalt-base, carbide-hardened alloy consisting essentially of cobalt and, in weight percent, about 19% to about 23% chromium, about 8 to about 12% nickel, about 0.5% to about 0.7% carbon, about 7% tungsten, about 3.5% tantalum, about 0.2% titanium and about 0.5% zirconium.

7. A precision cast, vacuum-melted, carbide-hardened alloy consisting, in weight percent, of about 0.6% carbon, about 21.5% chromium, about 10% nickel, about 7% tungsten, about 3.5% tantalum, about 0.2% titanium, about 0.5% zirconium with the balance being essentially cobalt.

8. A precision cast, carbide-hardened alloy consisting of about 0.5% to 0.7% carbon, about 19% to 23% chromium, about 8% to 12% nickel, about 6% to 9% tungsten, about 2% to 5% tantalum, zirconium and titanium in amounts such that the minimum percentage of titanium is about 0.1%, the maximum percentage of zirconium is 1% and the percentage of zirconium is about 2.5 times the percentage of titanium, up to about 3% iron, up to about 0.5% manganese, up to about 0.5% silicon, up to 0.1% boron, up to 0.2% mischmetal, up to 2% columbium, up to 2% molybdenum and the balance being essentially cobalt.

## References Cited

## UNITED STATES PATENTS

|           |        |                      |        |
|-----------|--------|----------------------|--------|
| 2,763,547 | 9/1956 | Dyrkacz et al. ----- | 75—171 |
| 2,920,956 | 1/1960 | Nisbet et al. -----  | 75—171 |
| 2,974,036 | 3/1961 | Thielemann -----     | 75—171 |
| 3,026,199 | 3/1962 | Thielemann -----     | 75—171 |

RICHARD O. DEAN, Primary Examiner.

U.S. Cl. X.R.

UNITED STATES PATENT OFFICE  
CERTIFICATE OF CORRECTION

Patent No. 3,432,294

March 11, 1969

Harold L. Wheaton

It is certified that error appears in the above identified patent and that said Letters Patent are hereby corrected as shown below:

Column 1, line 56, "an", first occurrence, should read -- the --. Column 2, line 46, "any" should read -- an --. Column 3, line 1, "mtlting" should read -- melting --; line 6, after "oxidation" insert a comma. Column 4, lines 32 and 33, "as a substitute for a part of the required tantalum" should read -- (niobium) is not the full equivalent of tantalum --; line 38, "substrate" should read -- substitute --; line 53, "0.0% carbon" should read -- 0.60% carbon --. Column 5, TABLE II, fourth column, line 1 thereof, "11.1" should read -- 102.1 --; same table II, in the heading to the fifth column thereof, "Elongation, percent (1" gauge length" should read -- Elongation percent (1" gauge length) --. Column 6, TABLE III, in the heading to the second column thereof, "Temperature °F.)" should read -- Temperature (°F.) --. Column 7, line 19, "fatigues" should read -- fatigue --; line 26, after "the" cancel "v.". same column 7, TABLE VI, in the heading to the second and third column thereof, line 4, "(K.s.i.)", each occurrence, should read -- K.S.I. --. Column 8, line 19, before "about", second occurrence, insert -- least --.

Signed and sealed this 7th day of April 1970.

(SEAL)

Attest:

EDWARD M.FLETCHER,JR.  
Attesting Officer

WILLIAM E. SCHUYLER, JR.  
Commissioner of Patents